

1

3,010,842

**DEVELOPMENT OF ELECTROSTATIC IMAGES**  
Eugene C. Ricker, Columbus, Ohio, assignor, by mesne assignments, to Xerox Corporation, a corporation of New York  
No Drawing. Filed Aug. 29, 1955, Ser. No. 531,280  
1 Claim. (Cl. 117—37)

This invention relates to a method for the development of electrostatic latent images.

In xerography it is usual to form an electrostatic latent image on a surface. One method of doing this is to charge a photoconductive insulating surface and then dissipate the charge selectively by exposure to a pattern of activating radiation. Other means of forming electrostatic latent images are set forth in U.S. 2,647,464 to James P. Ebert. Whether formed by these means or any other, the resulting electrostatic charge pattern is conventionally utilized by the deposition of an electrostatic material thereon through electrostatic attraction whereby there is formed a visible image of electroscopic particles corresponding to the electrostatic latent image. Alternatively, the electrostatic charge pattern may be transferred to an insulating film and the electroscopic particles deposited thereon to form the visible image. In any case, this visible image, in turn, may be transferred to a second surface to form a xerographic print.

The process of depositing the electroscopic powder on the electrostatic image to render the electrostatic image visible is called the "development step" and is one of the most critical steps of the entire process. As the electrostatic latent image is developed by deposition of an electroscopic material thereon, it is obvious that the process offers freedom from dependence on the awkward and complicated liquid development processes of conventional photography. To emphasise this freedom the process has been named xerography as generally dry powders were used as the electroscopic materials. However, this is not necessarily the case as is shown in U.S. 2,551,582 to C. F. Carlson wherein the electroscopic material was applied in the form of a liquid spray.

It is evident that no picture can be better than the development step permits. About the coarsest type of image reproduced by a xerographic process requires a resolution of at least about 50 lines per inch. Commercial line-copying xerographic machines generally have a resolution power of about 125 to 250 lines per inch. The process used in obtaining this resolution is termed cascade development and is set forth in U.S. 2,618,552. This process involves the use of a finely-divided colored material colored called a "toner" deposited on a slightly more coarsely-divided material called a "carrier." This two-component developer is cascaded across the electrostatic image areas.

The control of the concentration of toner in the two-component developer becomes difficult on continued operation of a xerographic machine. When applied to continuous-tone development where resolutions greater than about 300 lines per inch are necessary it has been found impossible to obtain the desired quality of reproduction using such a system. Accordingly, another system of xerographic development known as "powder cloud development" has been evolved. In this process a powder cloud is generated by agitating a mass of dry electroscopic material in a confined space or in the case of a liquid by spraying through an atomizer. The cloud so produced is charged and then contacted with the electrostatic latent image. This process makes possible the realization of extremely high resolutions such as 1200 or more lines per inch. Furthermore, concentration of toner is more susceptible to control so that the process is easily adaptable for use on continuous machines.

2

However, the process also has its defects. Thus, to realize the high resolutions possible with this system and to obtain solid-area coverage it is necessary to use a development electrode—that is a conductive electrode spaced close enough to the image-bearing surface to draw the lines of force externally above the image-bearing surface. Due to the low dielectric constant of air an extremely close spacing of the development electrode is desired for its effective use. This introduces a number of difficulties due to the extreme difficulty of obtaining adequate air flow in the very narrow and confined space between the development electrode and the image-bearing surface. Other difficulties arise in attempting to obtain a constant flow for extended periods of time from the powder cloud generator and in flowing a uniform powder cloud over all areas of the image-bearing surface. Moreover powder clouds are not uniformly charged to the same polarity—a significant portion of the cloud will be of the opposite polarity to that desired for the development of the image. These oppositely charged particles in the cloud tend to deposit from the powder cloud on uncharged areas of the image making difficult the obtaining of a clear white on such areas. Finally, the equipment for generating, charging and directing the flowing of the powder cloud becomes rather complicated.

The instant invention relates to a process which represents a substantial improvement in the art of xerographic development. In this process the electroscopic material is suspended in a liquid rather than a gas and the electrostatic latent image developed by contacting the image-bearing surface with the liquid suspension to produce a layer of liquid on the image-bearing surface whereby the electroscopic material is attracted out of the liquid to the image-bearing surface as by immersion of the image-bearing member in the suspension, by flowing the suspension over the image bearing surface or otherwise. This process has several advantages over the prior art: Thus, development is almost instantaneous. Contacting the liquid suspension of powder particles with the electrostatic image to form a layer of the liquid suspension thereon is easily and quickly accomplished without the necessity for complicated and cumbersome equipment. The particles are believed to be all charged with the same polarity (probably a zeta-potential) without the necessity for special charging equipment. The use of a liquid permits a higher concentration of useable developer particles than when gas is the suspending medium. The image defects due to irregularities in the air flow are obviated and, finally, the use of a liquid having a high dielectric constant permits more effective use of a development electrode.

The process of the invention will now be set forth in more detail.

According to the present invention a dispersion of electroscopic particles is formed in a suitable liquid for example as by stirring or otherwise as is well known to those skilled in the art. Suitable electroscopic particles include any pigment or similar material having a fine particle size and being insoluble in the suspending liquid. In general the finer the powder the better the grain in the developed image. It is preferred that the average particle size be no larger than about 20 microns and for high quality work it is preferred that the average particle size be no more than about 5 microns. Suitable materials readily available in the desired size range include charcoal, magnesium oxide, lithopone, cadmium yellow, chrome yellow, cobalt blue, sulfur, vermillion, barium yellow, cadmium red, ochre, burnt umber, cobalt green, burnt sienna, ultramarine blue, Hansa yellow, rose madder, Dupont Luxol blue, and methyl cellulose. As already mentioned the pigment should not be soluble in the liquid and it must also be so selected relative to the liquid used as to assume a charge of the desired polarity. The

electrostatic charge imparted to suspended particles is a function both of the nature of the particles and of the suspending liquid.

The liquid used must have a relatively high insulating value to avoid discharge of the latent electrostatic image. Suitable liquids include hydrocarbons such as benzene, xylene, hexane, naphtha, kerosene, etc.; halogenated hydrocarbons such as carbon tetrachloride, trichloroethylene, chloroform, Genetrons (a trade name of Allied Chemical Co. for various fluorinated compounds), Freons (a trade name of E. I. du Pont de Nemours & Co. for various fluorinated compounds), etc.; miscellaneous liquids such as turpentine, etc.

Any method known to those skilled in the art may be used for dispersing the pigment in the liquid. In general simple stirring or agitation of the liquid is sufficient. Where a highly uniform and stable suspension is desired, the suspension formed by stirring may be passed through a colloid mill, but excellent suspensions may be attained without such treatment. Suspending agents may be used where they do not impair the insulating properties of the liquid.

The density of pigment deposited on the xerographic plate is dependent on the charge of the electrostatic latent image, the pigment concentration in the liquid and the presence of a development electrode. As is the case in powder cloud development described above the development electrode consists of a conductive electrode, either of continuous conductive material as sheet metal or of a conductive foraminous grid, closely spaced to the image-bearing surface. The function of the development electrode is to draw the lines of force of the electrostatic image externally above the image-bearing surface. This gives improved solid-area coverage and, by increasing the amount of the lines of force that are external to the image-bearing surface and hence available to attract electrostatically charged marking particles, improves the overall efficiency of the development process. Where the liquid suspension is contacted with the electrostatic image-bearing surface in a conductive dish or tank, the walls of the container will themselves constitute a development electrode. Moreover, the use of liquids having much higher dielectric constants than air permits the effective use of a development electrode at considerably greater spacings from the image-bearing surface than when air is the intervening dielectric.

The developed images are satisfactory for visual inspection on the plate while still wet. If desired, the wet image may be transferred by absorption by paper. If desired, the image may be dried and transferred to a desired base such as paper, plastic, etc. by the usual methods of electrostatic transfer as described in U.S. 2,576,047 to R. M. Schaffert or adhesive transfer as described in U.S. 2,661,289 to Mayo and Wolfe. The image, in turn, may then be fixed by any means known to those skilled in the art such as those described, for example, in U.S. 2,297,691 to C. F. Carlson. Thus where either the pigment itself fusible by heat or solvent vapor, or where the sheet to which it is transferred is coated or impregnated with a material fusible by heat or solvent vapor, then the use of either heat or solvent vapor will permanently affix the image to the sheet. Alternatively, another method of fixing the image comprises spraying the surface of the sheet bearing the image with a fixative lacquer by atomizer. Other means of transferring and/or fixing the image known to those skilled in the art may be used.

In the following examples a xerographic plate comprising a 20 micron layer of selenium on an aluminum backing was charged and exposed to a pattern of light and shadow in a XeroX Copier and XeroX Camera Unit No. 1 commercially available from the Haloid Company of Rochester, New York. In each case the electrostatic latent image had a positive polarity.

#### Example 1

A liquid suspension of 1 g. of finely-divided talc in 100 cc. of naphtha was prepared by stirring with a steel rod. The xerographic plate was developed by pouring the suspension over the plate. A positive image was obtained of poor definition due to excessively thick deposits.

#### Examples 2-17

Liquid suspensions were prepared by dispersing 0.5 g. of each of the following materials in 100 cc. of naphtha and stirring with a steel rod. Development was as above.

| Example | Material             | Comments                                                 |
|---------|----------------------|----------------------------------------------------------|
| 2       | Sulphur              | No comment.                                              |
| 3       | Hansa Yellow         | Poor image.                                              |
| 4       | Charcoal             | Do.                                                      |
| 5       | Dupont Luxol Blue    | Good reversal development.                               |
| 6       | Rose Bengal          | Good positive development.                               |
| 7       | Powdered Brass       | Exceptionally good positive image.                       |
| 8       | Cobalt blue          | No comment.                                              |
| 9       | Yellow ochre         | Apparent reversal development.                           |
| 10      | American vermilion   | Apparent reversal development. Sharp and bright letters. |
| 11      | Burnt umber          | Positive image. Good solid area coverage.                |
| 12      | Lithopone            | Poor image.                                              |
| 13      | Burnt Sienna         | Positive image. Good solid area coverage. Quite sharp.   |
| 14      | Cadmium red          | No comment.                                              |
| 15      | Chrome yellow (med.) | Reversal development.                                    |
| 16      | Powdered aluminum    | Poor contrast and definition. Too much deposition.       |
| 17      | Methyl cellulose     | Poorly good continuous tone development.                 |

#### Example 18

A suspension was prepared by stirring 0.5 g. finely-divided charcoal into 100 cc. steam-distilled turpentine. An image was developed as in Example 1. Deposition was light.

#### Example 19

A liquid suspension was prepared by placing in a glass container 1.0 g. of finely-divided charcoal and 100 cc. of carbon tetrachloride. The container was then stoppered and dispersion completed by manually shaking a few times.

The suspension was then poured into a metal tray and the image-bearing surface contacted with the suspension by immersing the xerographic plate therein in the dark. The plate used in this example consisted of a 50 micron layer of selenium on a brass backing. After immersion the plate was withdrawn from the suspension, the lights turned on and the image transferred while wet by contact with dye-transfer paper. By this process a completely developed xerographic image was obtained in just a few seconds and with only the simplest of equipment.

#### Examples 20 and 21

Suspensions were prepared as in Example 1 using 0.1 g. finely-divided aluminum and 0.1 g. finely-divided copper, in each case dispersed in 100 cc. of naphtha. Development was in Example 1. Both produced good images, the aluminum having slightly better resolution.

#### Example 22

A suspension of 0.1 g. finely-divided charcoal in 100 cc. of carbon tetrachloride was prepared as in Example 1. The image was developed as in Example 1, and then transferred while wet by contact with dye-transfer paper. The print so produced had exceptionally high quality, both on continuous tone and on line copy.

#### Example 23

A suspension was prepared by stirring  $\frac{1}{2}$  teaspoon of an alcohol "dag" obtained from Acheson Colloids, Port Huron, Michigan, into 120 cc. of naphtha. The image was developed as in Example 1. The image was thin due to light deposition.

*Examples 24 and 25*

Suspensions were prepared as in Example 1 using 0.5 g. of charcoal and 0.25 g. of aluminum powder, in each case dispersed in 100 cc. of xylene. The images were developed as in Example 1. Fair images were obtained.

*Example 26*

A suspension was prepared by stirring both 0.1 g. of charcoal and 0.1 g. of aluminum powder into 100 cc. of naphtha. The image was developed as in Example 1. The developed image was a mixture of both the charcoal and the aluminum.

The increased versatility of xerography due to the availability of such alternative development processes is obvious at once. Thus it is possible to develop an image either positively or negatively by selecting a liquid-pigment system wherein the charge on the particles is, respectively, either opposite to or the same as the polarity of the charge of the electrostatic image. Furthermore, it is possible to produce images of mixed colors by blending pigments of different color but similar charge polarity. It is also possible to simultaneously develop both the image and the background by using two pigments which take on the opposite polarity of charge when dispersed in the same liquid. While a particular embodiment of the invention has been described, it is not intended to be limited thereto, but it is intended to cover the invention broadly within the spirit and scope of the appended claim.

## I claim:

A process of developing an electrostatic latent image on an insulating surface which comprises contacting an electrically insulating layer bearing an electrostatic latent

image with an electrically insulating liquid so that all of the image-bearing portions of said layer contact said liquid, said liquid having dispersed therein finely-divided particles of a first color and finely-divided particles of a second color, the particles of said first color and the particles of said second color having opposite polarities as a result of being dispersed in said liquid, and simultaneously developing both the image and background on said insulating layer.

10

## References Cited in the file of this patent

## UNITED STATES PATENTS

|           |                |               |
|-----------|----------------|---------------|
| 1,174,903 | Schwerin       | Mar. 7, 1916  |
| 1,589,327 | Eberlin et al. | June 15, 1926 |
| 1,870,408 | Dreyfus et al. | Aug. 9, 1932  |
| 2,251,992 | Flory et al.   | Aug. 12, 1941 |
| 2,297,691 | Carlson        | Oct. 6, 1942  |
| 2,633,796 | Pethick        | Apr. 7, 1953  |
| 2,761,416 | Carlson        | Sept. 4, 1956 |
| 2,784,109 | Walkup         | Mar. 5, 1957  |
| 2,808,328 | Jacob          | Oct. 1, 1957  |

## FOREIGN PATENTS

|         |               |               |
|---------|---------------|---------------|
| 698,994 | Great Britain | Oct. 28, 1953 |
|---------|---------------|---------------|

## OTHER REFERENCES

Metcalfe: "Liquid Developers for Xerography," Journal of Scientific Instruments, vol. 32, February 1955, pp. 74 and 75.

Atkinson et al.: "Ferrography," Journal of the Franklin Institute, vol. 252, No. 5, November 1951 pp. 373-381.